

# United States Patent [19]

Vellins et al.

[11] 3,893,801

[45] July 8, 1975

[54] TRANSFER DYEING

[75] Inventors: Cyril Eric Vellins, Cheadle; Leonard Fox Dixon, Elland; Bryan Ronald Hinchliffe, Huddersfield, all of England

[73] Assignee: L. B. Holliday & Co. Limited, Huddersfield, England

[22] Filed: June 14, 1973

[21] Appl. No.: 369,970

[52] U.S. Cl. .... 8/2.5; 8/39; 8/2.5

[51] Int. Cl. .... D06p 1/20

[58] Field of Search ..... 8/2.5, 39

[56] References Cited

UNITED STATES PATENTS

1,938,029 12/1933 Kugel ..... 260/378  
3,707,346 12/1972 Markert et al. .... 8/39

FOREIGN PATENTS OR APPLICATIONS

359,850 10/1931 United Kingdom ..... 8/39

OTHER PUBLICATIONS

Fox et al., Dec. 1969, J. Soc. Dyers & Col., pp. 614-616.

Primary Examiner—Donald Levy

Attorney, Agent, or Firm—William R. Liberman, Esq.

[57]

## ABSTRACT

A method for transfer printing onto a synthetic fabric is provided utilizing an ink comprising a base medium and at least one dyestuff having the formula:



in which: X is an unsubstituted alkyl group having from 1 to 6 carbon atoms, Y and Z are cyano or hydrogen, at least one of Y and Z being cyano.

12 Claims, No Drawings

## TRANSFER DYEING

This invention relates to transfer dyeing or printing.

According to our invention we provide a method of transfer printing in which an ink comprising a base medium, and at least one dyestuff of formula (I)



in which:

X is an alkyl group having from 1 to 6 carbon atoms which may be substituted, or a cycloalkyl group containing 6 carbon atoms, Y or Z is cyano or hydrogen or both Y and Z are cyano; is printed in a desired design, alone or together with one or more other dyestuffs, on to a transfer backing material, and in which the printed design is thereafter transferred from the backing material to a synthetic material which is to be dyed or printed by the application of heat.

According to one aspect of our invention, we provide a method of transfer printing in which an ink comprising a base medium and at least one dyestuff of formula (I):



in which:

X is an alkyl group having from 1 to 6 carbon atoms which may be substituted or a cycloalkyl group containing 6 carbon atoms, Y is cyano or hydrogen and Z is cyano.

is printed in a desired design, alone or together with one or more other dyestuffs, on to a transfer backing material, and in which the printed design is thereafter transferred from the backing material to a synthetic material which is to be dyed or printed by the application of heat.

In general, the transfer backing material containing the printed design is contacted with the synthetic material which is to be dyed and heated at a temperature in the range of from 180° to 230°C. for a period of from 10 seconds to 2 minutes, preferably from 15 seconds to 30 seconds, but the precise conditions will depend on the materials employed and the desired results.

The transfer printing process involves the conversion to the vapour phase by heat of the dyestuff which has been previously printed onto an inert support, followed by penetration and adsorption into the synthetic material to be dyed.

Suitable alkyl or cycloalkyl groups represented by X in formula (I) above are saturated alkyl groups such as methyl, ethyl, normal or isopropyl, butyl or cyclohexyl.

Specific examples of compounds of formula (I) are 5 1-amino-2-cyano-4-methylaminoanthraquinone, 1-amino-3-cyano-4-cyclohexylaminoanthraquinone, 1-amino-2,3-dicyano-4-methylaminoanthraquinone, 1-amino-2,3-dicyano-4-ethylaminoanthraquinone and 1-amino-2,3-dicyano-4-n-butylaminoanthraquinone.

10 The design may be printed on the backing material, normally paper, by any of the usual paper printing processes such as a flexographic, lithographic, gravure, letter press or screen printing process. The printing ink is formulated to be suitable for the desired process, but 15 in general is made up of one or more solvents, a resinous or oily binding and thickening material, and the desired dyestuff, either in finely divided form or wholly or in part in solution. The binding material should not decompose or transfer at the required transfer temperature.

20 Mixtures of dyes of formula (I) may be used to give, in some cases, greater depths of shade. If the cyano compounds are prepared by the processes described in U.S. Pat. No. 1,938,029, natural mixtures result which 25 are commercially attractive.

One possibility is to have substantially equal amounts of 2-cyano and 3-cyano derivatives. Another is to have a preponderance of 2,3-dicyano compound and only small amounts of the 2-cyano and 3-cyano compounds.

30 The following examples illustrate the application of the process.

## EXAMPLE 1

35 20 g of 1-amino-4-butylamino anthraquinone-2-sodium sulphonate, 25 g of potassium cyanide, 5 g sodium carbonate and 1000 g of water are heated to 80°-90°C. until the product has completely precipitated from the original blue solution. The reaction mixture is then filtered, washed with water and dried to 40 give a mixture of 1-amino-2,3-dicyano-4-butylaminoanthraquinone mixed with small amounts of the corresponding 2 and 3 mononitriles.

45 5 parts of the above dye mixture are ground to a fine dispersion in a ball mill with 95 parts of the following solution:

50 parts of shellac  
50 parts of methylated spirits (64 o.p.)  
8.5 parts of monoethanolamine  
3.5 parts of morpholine  
0.3 parts of silicone antifoam agent  
15 parts water

50 The ink may be printed by flexographic roller onto a paper base, dried, and the paper contacted with a polyester fabric at 215°C. for 20 seconds. The resulting 55 clear blue dyeing has good fastness to washing and light. Good prints may be obtained on other synthetic fibres and films, such as nylon and acrylic di- and triacetate. On the latter fibres, gas fume fastness is also excellent.

60

## EXAMPLE 2

A mixture of 22 parts of modified phenolic resin, e.g. 65 Alsynol RL 23, and 48 parts of bleached linseed oil is heated to 260°C. and thereafter cooled to 190°C. 30 Parts of linseed oil modified alkyd resin, e.g. Alsynol PN 53 are added, the mixture being cooled to 40°C. when 15 parts of the dye of example 1 are added and

the mixture is milled. After the addition of 6 parts of 6% cobalt naphthenate (6% cobalt), an ink suitable for offset or litho printing on paper is produced. Heat transfer to fabric gives similar results of example 1.

### EXAMPLE 3

A mixture of 150 g 1-amino-4-bromoanthraquinone-2-sodium sulphonate, 96 g 60% aqueous ethylamine solution, 20 g sodium carbonate, 0.75 g copper acetate and 1000 ml water is heated in a stainless steel autoclave at 95°-100°C. for 3 hours. Excess ethylamine is removed by venting and the solution of 1-amino-4-ethylaminoanthraquinone-2-sulphonic acid is further diluted to 3 litres with water. 144 g sodium cyanide and 25 g sodium carbonate are then added and the mixture is heated to reflux until the product has precipitated. The dye is then filtered, washed with hot water and dried, to give a mixture of mainly 1-amino-4-ethylamino-2,3-dicyano anthraquinone, together with small amounts of the corresponding 2 and 3 monocyano derivatives.

50 parts of the above dye and 50 parts of hydroxypropyl cellulose are sand ground with water to a fine dispersion, and then spray dried. 12 parts of the above mixture with 5 parts of ethyl cellulose are mixed with 78 parts of isopropanol. The resulting ink when coated on paper gives good bright blue heat transfer prints when transferred as in Example 1.

This dye may be converted to an ink equally well by the processes used in Examples 1 and 2.

### EXAMPLE 4

A mixture of 20 g of 1-amino-4-cyclohexylamino anthraquinone-2-sodium sulphonate, 40 g of potassium cyanide and 1000 ml of water are refluxed for 2 hours, filtered, washed and dried. The product is mainly 1-amino-3-cyano-4-cyclohexylaminoanthraquinone. 5 parts of a 50% mixture of this dye with 50% ethyl cellulose (prepared similarly to example 3) were diluted with 45 parts of methylethylketone and 45 parts of ethanol, and the viscosity was adjusted by addition as necessary of ethyl cellulose to give an ink suitable for rotogravure or heliogravure.

Transfer prints on to synthetic fibres were a bright reddish blue of good wash and light fastness. The results were equally good when applied from ink coated paper prepared with inks as in the previous examples.

### EXAMPLE 5

20 g of 1-amino-4-methylaminoanthraquinone-2-sodium sulphonate, 25 g of potassium cyanide, 5 g of sodium carbonate and 1000 ml water are heated at 85°-95°C. for 3 hours. The mixture is filtered, washed with hot water and dried, to give a mixture of cyano derivatives which is mainly 1-amino-2-cyano-4-methylaminoanthraquinone. A mixture of 20 parts of the above dye, 30 parts of calcium carbonate extender, 12.5 parts of long oil linseed isophthalic acid alkyd resin, 25 parts of medium viscosity linseed oil and 12.5 parts of heavy viscosity linseed oil is passed through a triple roll mill to give an offset litho ink. Papers so printed gave good heat transfer prints on synthetic fibres.

### EXAMPLE 6

A mixture of equal parts of the dyestuffs of Examples 1 and 5 was made into an ink and printed as in Example

1. Deeper blue shades on transfer printing were obtained than by the use of either dye singly.

We claim:

1. A method of transfer printing comprising printing with an ink a desired design onto a transfer backing material, and thereafter transferring the printed design by the application of heat from the backing material to a synthetic fabric which is to be dyed or printed, the ink comprising a base medium and at least one dyestuff 10 having the formula



in which: X is an unsubstituted alkyl group having from 1 to 6 carbon atoms, Y and Z are cyano or hydrogen, at least one of Y and Z being cyano.

2. A method of transfer printing comprising printing with an ink a desired design onto a transfer backing material, and thereafter transferring the printed design by the application of heat from the backing material to a synthetic fabric which is to be dyed or printed, the ink comprising a base medium and at least one dyestuff having the formula



in which: X is an unsubstituted alkyl group having from 1 to 6 carbon atoms; Y is cyano or hydrogen and Z is cyano.

3. A method according to claim 2 in which the transfer backing material containing the printed design is contacted with the synthetic fabric to be dyed and heated at a temperature in the range of from 180° to 230°C. for a period of from 5 seconds to 1 minute.

4. A method according to claim 3 in which the heating period is for from 5 seconds to 30 seconds.

5. A method according to claim 1 in which the saturated alkyl group is methyl, ethyl, normal propyl or isopropyl or butyl.

6. A method according to claim 1 in which the compound (I) is 1-amino-2-cyano-4-methylaminoanthraquinone.

7. A method according to claim 2 in which the saturated alkyl group is selected from the group consisting of methyl, ethyl, normal propyl, isopropyl or butyl.

8. A method according to claim 2 in which mixtures of two or more compounds (I) are employed.

9. A method according to claim 1 in which the compound (I) is 1-amino-2,3-dicyano-4-methylaminoanthraquinone.

10. A method according to claim 1 in which the compound (I) is 1-amino-2,3-dicyano-4-ethylamino anthraquinone.

11. A method according to claim 1 in which the compound (I) is 1-amino-2,3-dicyano-4-n-butylamino an-

thraquinone.

12. A method according to claim 1 in which mixtures of two or more compounds (I) are employed.

\* \* \* \* \*